

June 16, 1959

S. A. HAYS

2,890,944

CONTINUOUS CHEMICAL MILLING PROCESS

Filed May 25, 1956



INVENTOR.  
STEPHEN A. HAYS

BY

*William R. Hays*

ATTORNEY

1

2,890,944

**CONTINUOUS CHEMICAL MILLING PROCESS**

Stephen A. Hays, La Mirada, Calif., assignor to North American Aviation, Inc.

Application May 25, 1956, Serial No. 587,418

17 Claims. (Cl. 41—42)

This invention relates to improvements in the process for chemically milling group VIII metals and alloys thereof. More specifically, this invention relates to a chemically milling process for metals which can be controlled to produce finished products of uniform quality.

Processes have recently been developed for chemically milling steel. These processes involve contacting a steel workpiece with an acid chemical milling solution for a period of time sufficient to remove a desired amount of metal from the exposed surface of the steel workpiece. The method employed in the past has consisted of a batch process, that is, an acid solution of a particular strength was made up and steel workpieces subjected to its action for a given period of time. During this period, the strength of the solution was gradually depleted. When the strength of the solution became too low for chemical milling, the solution was discarded and a new solution was made up. The prior art processes, however, contain a number of disadvantages. One disadvantage is that the effectiveness of the milling solution is often exhausted in a short period of time requiring interruption of the process while new solutions are prepared. On a commercial scale, the cost of such a procedure is often prohibitive. A characteristic disadvantage of the batch process is that the strength of the solution is very high at the beginning of the chemical milling and decreases to minimum effectiveness as the milling progresses. This makes it very difficult to control not only the rate of the chemical milling, but also the quality of the chemically milled surface. For instance, when the acid concentration of the solution is high, a very rough surface is obtained on the part exposed to the solution. Likewise when the solution has become run down or too low in acid concentration, a poor or rough surface is also obtained. Still another problem in the prior art batch process is the disposal of the spent chemical milling solutions. The acid, nitrate and metal content of the waste solutions prohibit direct disposal in sewage systems. Alkaline neutralization is costly and still leaves a high nitrate solution which, also, may not be disposed of through the sewage systems. It is thus seen that a need exists for a process of chemically milling metals such as steel and steel alloys which not only can be controlled so as to provide finished articles of uniform quality, but also will eliminate the waste disposal problem.

It is therefore an object of the present invention to provide a chemical milling process which can be used for chemically milling group VIII metals and alloys thereof. It is also an object of this invention to provide a chemical milling solution by the use of which the quality of the chemically milled surface of steel and steel alloy workpieces may be controlled. Another object of this invention is to provide a process for controlling the composition of a chemical milling solution. It is likewise an object of this invention to provide a chemical milling process by the use of which the quality of the chemically milled surface may be controlled. Another object of this

2

invention is to provide a process which eliminates waste disposal problems. The above and other objects of invention will become more apparent from the discussion that follows.

5 The above and other objects of the invention are accomplished by a continuous process of chemically milling workpieces of group VIII metals and alloys thereof comprising exposing a workpiece to the etching action of a chemical milling bath initially containing dissolved phosphorus and metal in a predetermined weight ratio, wherein the phosphorus is present in the form of soluble phosphates, withdrawing partially spent portions of the bath containing the dissolved metal and phosphorus, and adding phosphorus in the form of soluble phosphates to the bath in an amount substantially equivalent to the phosphorus removed in the partially spent portions. By carrying out the process in this manner, the concentration of phosphorus and metal in solution is thus maintained within a predetermined range of values and provides a method for obtaining workpieces having smooth chemically milled surfaces from which the metal has been removed to an even depth.

20 The steel and steel alloys that can be chemically milled by the process of this invention includes metal alloys having very low percentage of steel by weight. For example, the process can be applied to milling Inconel "X" which contains only 7 weight percent iron and 75 weight percent nickel, together with other elements. The complete composition of Inconel "X" is given in 25 Bulletin T-7 entitled "Engineering Properties of Inconel and Inconel 'X,'" issued by the International Nickel Company, Inc., New York, in June 1953. It can also be applied to milling Invar which contains 36 weight percent nickel and 64 weight percent steel. Generally, the process is applicable to chemically milling the metals of group VIII of the periodic table of elements and their alloys.

30 The dissolved phosphorus is present in the form of soluble phosphates such as phosphoric acid and metal phosphates including soluble metal hydrogen phosphates. Examples of such phosphates are phosphoric acid, ferric phosphate and its hydrates, the hydrogen phosphates of iron such as  $Fe_2(HPO_4)_3$  and  $Fe(H_2PO_4)_3$ , chromic phosphates and its hydrates, chromic hydrogen phosphates, nickel phosphate, nickel hydrogen phosphates, etc. The dissolved metal is present in the form of metal salts such as the metal phosphates named above or the soluble nitrate and chloride salts of the metals. Hence, the dissolved metal will be present in solution in the form of metal ions. The kind of metal in solution will depend to a large extent on the composition of the metal workpieces subjected to the action of the chemical milling bath and includes metals such as iron, nickel, chromium, 35 cobalt, as well as small amounts of various metal impurities found in steel and its alloys.

40 The single figure of the drawing represents a flow sheet of the process.

An embodiment of this invention comprises precipitating metal phosphates from the partially spent portions 45 which have been withdrawn from the chemical milling bath, leaving an effluent or liquid phase containing metal hydrogen phosphates, and returning the liquid phase which contains the metal hydrogen phosphates back to the bath. The only amount of phosphorus in the form of soluble phosphates that need be added in this case is that equivalent to the amount precipitated as metal phosphates from the withdrawn portion. Since the process is applicable to the chemical milling of steel and its alloys, the metals going into the solution will include not only iron but also other metals such as chromium, nickel, cobalt, etc. Hence the metal phosphates which

are precipitated from the withdrawn partially spent portions of the chemical milling bath comprise a mixture of the phosphates of the various metals of which the workpiece consists, i.e., phosphates of iron, nickel, cobalt, chromium, etc. In like manner the effluent which is returned to the milling bath will contain hydrogen phosphates of these metals.

Ingredients of the bath which are lost by reaction and evaporation, or removed in the withdrawn portions, are replaced by the additions of the respective ingredients to the bath.

The purpose of the precipitation is to remove excess metal from the milling solution. Returning the effluent to the milling bath provides for the utilization of all the other components of the milling solution. Thus the process provides a chemical milling method which not only results in controlled removal of metal from the exposed surface of a workpiece, but also minimizes waste of bath components and results only in a metal phosphate by-product.

The other components of the chemical milling bath are comprised of hydrohalic acid and/or nitric acid together with water. Small amounts of other components including inorganic and organic acids such as sulfuric acid, nitrous acid, acetic and other organic acids may also be present either as impurities or they may be added to modify the chemical milling solution.

The dissolved phosphorus-to-metal weight ratio in the milling solution can vary from about 0.23 to about 1.50. When the ratio is maintained within this range, it is found that the process readily lends itself to control of the rate at which the metal is chemically removed from the surface exposed to the milling solution. The metal is removed to a uniform depth over the entire exposed surface. Also, a smooth chemically milled surface is obtained regardless of the amount of metal removed per unit area. Since the ferric and other metal phosphates which are precipitated from the effluent are the only by-products of the process, the previously encountered acid disposal problem is overcome. Furthermore, since phosphates are well-known articles of commerce, the process of this invention not only eliminates the wastes inherent in prior art processes but also produces a usable by-product.

An embodiment in the practice of this invention is the use of a combination of nitric, and hydrohalic acid such as hydrochloric and/or hydrofluoric acid, in the milling solution together with phosphoric acid and dissolved metal. When employing such a solution for chemical milling of steel and steel alloy workpieces, the total acid content of the chemical milling solution as well as the amount of halide, nitrate, phosphate and metal ions should also be kept within certain ranges in order to obtain a chemically etched surface of good quality. Therefore, an embodiment of this invention is a process for chemically milling steel and steel alloy workpieces comprising contacting said workpieces in a milling vessel with an acid chemical milling bath or solution containing 3.5-12.3 grams per liter of acidic hydrogen, 35.5-302 grams per liter of chloride ion, 80.5-279 grams per liter of nitrate ion, 43-172 grams per liter of phosphorus in the form of soluble phosphates, 30-200 grams per liter of dissolved metal, the balance being substantially water, and wherein the ratio by weight of phosphorus-to-dissolved metal is from about 0.23 to about 1.50; withdrawing partially spent portions of said solution having said predetermined phosphorus-to-dissolved metal weight ratio; precipitating metal phosphates from the withdrawn portions leaving a liquid phase containing metal hydrogen phosphates; returning the liquid phase containing metal hydrogen phosphates to the milling bath, and adding phosphorus in the form of soluble phosphates to the bath in an amount substantially equivalent to the phosphorus removed in the form of the metal phosphate precipitate.

One method of precipitating the metal phosphates from

the withdrawn portion is to first distill the withdrawn portion to produce a distillate of water, a distillate of hydrochloric plus nitric acids, and a residue containing phosphates of metal. Water is then added to residue to precipitate metal phosphates leaving an aqueous solution containing hydrogen phosphates of metal. The solution is separated from the precipitate and returned to the milling vessel. The solution or effluent may be condensed by distilling or evaporating to remove excess water, if any.

Small amounts of the various acids and water are usually lost in carrying out the process by evaporation, distillation and reaction. To compensate for this, additions of the various components of the bath may be made from time to time in order to replace those lost.

The general method of carrying out the process of this invention may be more readily explained by reference to the accompanying diagram. In this diagram a steel workpiece 1 has its edge 2, as well as the reverse side of the workpiece, masked with a suitable acid resistant material. The workpiece 1 is suspended by means of lines 3 which are likewise coated with a suitable acid resistant maskant, in a chemical milling solution 4 contained in a milling vessel 5. The milling vessel is constructed of an acid resistant material and is equipped with heating and cooling means as well as a temperature control means not shown in the diagram. A portion of the acid milling solution which contains phosphoric acids and dissolved metal is withdrawn through line 6 by cracking valve 7 and is admitted into a distillation apparatus 8. This withdrawn portion is progressively distilled to separate water and acids other than phosphoric such as hydrohalic and nitric acids, leaving a residue containing phosphates of iron and other metals. The residue may also contain some phosphoric acid which has not been used up in the formation of phosphates of iron. The water is taken off through line 9, and collected in water container 11. The water is taken off at temperatures of up to about 103° C. and the rate to which it is taken off is controlled by the valve 10. When hydrohalic and nitric acids are employed in the bath, they are also distilled off at temperatures of up to about 130° C. and are taken off through line 12, controlled by valve 13 and condensed in condenser 14. From the condenser, these acids are readmitted to the milling vessel through valve 15, thus completing the cycle for the hydrohalic and nitric acids. The residue containing phosphates of iron and other metals is withdrawn from the distilling apparatus through valve 16 and admitted to a precipitation vessel 17. Water, supplied from an outside source 39 to tank 11, is admitted through valve 19 in line 18 to the precipitation vessel 17. Ferric phosphate and other metal phosphates precipitate from the diluted solution, leaving hydrogen phosphates of iron and other metals in the solution. To aid in the precipitation of metal phosphates, heat can be applied to bring the contents of the precipitation vessel to, and maintain them at, the boiling point. The slurry of metal phosphate precipitate and metal hydrogen phosphates is next passed through valve 20 and filter 21. The metal phosphate precipitate is removed from the solution and the aqueous metal hydrogen phosphates, together with any free phosphoric acid that may be present, are conducted through valve 23 in line 22 into a concentration vessel 24. Heat is applied to the concentration vessel and its contents to distill or evaporate off excess amounts of water. The water distillate is taken off through valve 26 in line 25 and condensed and collected in the container 11. Alternatively, the water vapor may be vented to the atmosphere. The concentrated metal hydrogen phosphates are withdrawn from the concentration vessel through valve 27 and are conducted with the aid of pump 28 through line 29 back to the chemical milling vessel 5. Thus, by means of this process, metal removed from the workpiece 1 is precipitated as metal phosphates, while

all the other components of the chemical milling solution are returned to the milling vessel. To replace the phosphate removed in the precipitate, an equivalent amount of phosphoric acid is added to the milling vessel from the container 30 through valve 31 and line 38. Any water, hydrohalic acid and nitric acid which is lost in the various steps of the process or by evaporation and/or reaction, is replaced from the containers 32, 34 and 36 by manipulating the proper valves 33, 35 and 37 connected to the line 38 which leads to the milling vessel. Container 34 marked HX contains hydrohalic acid such as hydrochloric acid and/or hydrofluoric acid.

The rate at which the chemical milling solution is withdrawn through line 7 depends on the amount of metal surface exposed to access of the chemical milling solution. The rate of distillation of the withdrawn portion in the distilling apparatus 8 is adjusted to handle the amount of solution withdrawn. When the temperature of the acid vapors taken off reaches about 130° C., substantially all of the hydrochloric and nitric acids have been removed from the withdrawn portion. The residue containing the phosphates of iron and other metals may be continuously withdrawn through valve 16 to prevent a buildup in the distillation apparatus. This is preferred to an intermittent withdrawal although the latter is also practiced with good success. The precipitation in the vessel 17 may, likewise, be carried on either batchwise or continuously. The continuous process is preferred where a large amount of metal is being dissolved per unit volume of chemical milling solution per unit time since it is necessary to continuously withdraw the excess iron from the solution and to replace the phosphoric acid which is used up.

The point at which the excess water has been removed from the filtrate which contains the hydrogen phosphates of iron in concentrator 24, may be determined by the temperature of the distillate. When the temperature of the distillate has reached substantially 105° C., the metal hydrogen phosphates are sufficiently concentrated for return to the chemical milling vessel. Alternatively, the milling bath level, which varies with evaporation, deletions through line 6, and additions through line 38, may be maintained by adding solution from the concentrator 24 regardless of its concentration. Then, only the excess water need be evaporated from the solution containing the metal hydrogen phosphates. This may be accomplished by maintaining a maximum level in the concentrator. A float-controlled heater switch in the concentrator is one way of controlling the evaporation of the excess water.

The acid content of the milling solution is checked periodically by analysis for nitrate and chloride ion. The chloride ion is determined by a modified argentometric titration according to the method given in *Volumeetric Analysis*, volume II, by Kolthoff and Stenger, 1942 edition, page 242, Interscience Publishers, Inc., New York, with the modification consisting of the use of an electrometric end point. The nitrate ion determination is preceded by a basic precipitation of the metal from the sample. Following this, an analysis of the filtrate is conducted according to the method described in *Scott's Standard Method of Chemical Analysis*, 5th edition, by N. H. Furman, published by D. Van Nostrand of New York, vol. I, page 649.

The amount of phosphoric acid to be added can be determined from the weight of metal phosphates removed as precipitate. If desired, the amount of phosphate in the milling solution can also be determined by chemical analysis according to the method described in volume I of *Scott's Standard Method of Chemical Analysis*, 5th edition, page 697.

The following nonlimiting examples illustrate the processes of this invention in which the acidic hydrogen is defined as the hydrogens from the hydrohalic acid, nitric

acid and all three hydrogens from the phosphoric acid added to the bath, less the amount liberated due to reaction. The amount liberated is measured by the equivalence of metal dissolved.

#### EXAMPLE I

To the milling vessel of an apparatus of the type shown in the figure, was added water, phosphoric acid, nitric acid and hydrochloric acid in amounts such as to make up a solution containing 113 grams per liter of phosphorus in the form of soluble phosphate, 61 grams per liter of chloride ion and 108 grams per liter of nitrate ion. A sample of 17-7 pH steel containing 17 weight percent chromium and 7 weight percent nickel was then suspended in the chemical milling solution and the solution allowed to act thereon until the concentration of metal in solution reached 106 grams per liter as determined by the loss of weight of the steel sample. During the build up of the metal in solution, hydrochloric acid and nitric acid were added in amounts equivalent to 178 grams per liter of  $\text{NO}_3^-$  ion and 43 grams per liter of  $\text{Cl}^-$  ion. Some nitric and hydrochloric acids were lost due to reactions and evaporation. The concentrations of  $\text{NO}_3^-$  ion and  $\text{Cl}^-$  at this point were 148 grams and 92 grams per liter respectively. A 17-7 pH steel workpiece with masked edges was then suspended in the vessel allowing the chemical milling solution to act on the free surface. As the chemical milling of the workpiece progressed, a portion of the milling solution was continuously withdrawn and processed according to the procedure described hereinabove, with return of hydrochloric and nitric acids and of hydrogen phosphates of iron, chromium and nickel. The nitric, hydrochloric and phosphoric acids used up in the process were replaced by additions of appropriate amounts of the respective reagents. The workpiece was chemically milled to a depth of .070 inch at the rate of .020 inch per hour. The workpiece was then removed and washed with water. The surface of the chemically milled portion of the workpiece was smooth and chemically milled to an even depth. The weight ratio of phosphorus-to-iron in this example was 1.08, while the concentration of acidic hydrogen was about 9.6 grams per liter.

Equally good results were obtained when the chemical milling solution was prepared by adding 204 grams phosphoric acid reagent containing 85 percent acid by weight, 256 grams of hydrochloric acid reagent containing 37 percent acid by weight, 214 grams of nitric acid reagent containing 70 weight percent acid and 354 grams of ferric orthophosphate dihydrate per each liter of chemical milling solution to be prepared, the balance being substantially water. Thus, the weight ratio in solution of phosphorus-to-iron of 1.08 was directly obtained without requiring the solution to act on a piece of steel until the desired amount of metal had been dissolved.

#### EXAMPLE II

The procedure of Example I is repeated with a solution containing 30 grams per liter of iron, 43 grams per liter of phosphorus in the form of phosphoric acid, 35.5 grams per liter of chloride ion and 110 grams per liter of nitrate ion. The phosphorus-to-metal weight ratio in solution in this case is 1.50 and the acidic hydrogen concentration is 5.5 grams per liter. A workpiece of 17-7 pH steel exposed to this chemical milling solution for a period of four hours is chemically milled to a depth of substantially .080 inch, producing an even and smooth surface.

#### EXAMPLE III

A chemical milling solution containing 200 grams of iron per liter, 172 grams of phosphorus per liter in the form of phosphoric acid, 142 grams of chloride ion per liter and 105 grams of nitrate ion per liter is employed in the process described in Example I in milling workpiece of 316 Cres steel for a period of four hours to pro-

duce chemically milled surfaces of smooth and even quality. The weight ratio of phosphorus-to-metal in solution in this case is 0.90 and the acidic hydrogen concentration is 12.3 grams per liter. The Cres steel in this case contains about 18 weight percent chromium and about 13 weight percent nickel.

#### EXAMPLE IV

A chemical milling bath containing 200 grams of iron, 43 grams of phosphorus in the form of phosphoric acid, 302 grams of chloride ion and 80.5 grams of nitrate ion per liter of solution is employed to mill a workpiece of 17-7 pH steel. The exposed surface is chemically milled to a uniform depth. The weight ratio of phosphorus-to-metal in solution in this case is 0.23, while the acidic hydrogen concentrations are 3.5 grams per liter.

Other nonlimiting examples of composition of chemical milling solutions of this invention employed for chemically milling steel and steel alloy workpieces are given in the following table.

Table I.—Concentration in grams/liter  
PRODUCTS ACCEPTABLE

| No. | Workpiece     | Acidic H | Cl <sup>-</sup> | NO <sub>3</sub> <sup>-</sup> | P   | Metal | P/M Wt. Ratio | Rate of milling, inch/hr. | Time, Hrs. | Remarks                 |
|-----|---------------|----------|-----------------|------------------------------|-----|-------|---------------|---------------------------|------------|-------------------------|
| 1.  | 17-7 pH Steel | 6.2      | 220             | 105                          | 113 | 191   | 0.59          | .020                      | 1.0        | Smooth uniform surface. |
| 2.  | do            | 8.5      | 192             | 149                          | 113 | 190   | 0.59          | .020                      | 1.0        | do.                     |
| 3.  | do            | 10.6     | 50              | 124                          | 158 | 150   | 1.05          | .012                      | 1.3        | do.                     |
| 4.  | do            | 5.9      | 163             | 180                          | 45  | 112   | 0.40          | .037                      | 0.6        | do.                     |
| 5.  | do            | 9.9      | 112             | 105                          | 113 | 110   | 1.03          | .020                      | 1.5        | do.                     |
| 6.  | do            | 10.6     | 96              | 180                          | 113 | 110   | 1.03          | .047                      | 1.6        | do.                     |
| 7.  | do            | 9.6      | 92              | 114                          | 113 | 106   | 1.07          | .020                      | 3.5        | do.                     |
| 8.  | do            | 9.8      | 71              | 110                          | 113 | 91    | 1.24          | .023                      | 4.0        | do.                     |
| 9.  | 4130 Steel    | 11.3     | 35              | 279                          | 113 | 96    | 1.18          | .080                      | 4.0        | do.                     |
| 10. | Inconel "X"   | 11.5     | 153             | 290                          | 68  | 76    | 0.90          | .090                      | 0.5        | Smooth shiny surface.   |

PRODUCTS UNACCEPTABLE

|     |               |      |     |     |     |     |      |      |     |                                              |
|-----|---------------|------|-----|-----|-----|-----|------|------|-----|----------------------------------------------|
| 11. | 17-7 pH Steel | 17.1 | 199 | 204 | 113 | 109 | 1.04 | .042 | 1.0 | Extremely uneven surface with deep channels. |
| 12. | do            | 11.7 | 71  | 320 | 113 | 111 | 1.02 | .017 | 2.0 | Rough pitted surface.                        |
| 13. | do            | 11.9 | 100 | 93  | 113 | 63  | 1.79 | .023 | 2.0 | Wavy, scaly surface.                         |

In the above table letter P denotes phosphorus and M represents metal. Therefore, "P/M wt. ratio" represents the phosphorus-to-metal weight ratio in the solution. The 17-7 pH steel used in the examples contains about 73 weight percent iron, 17 weight percent chromium, 7 weight percent nickel, together with small amounts of other impurities. The 4130 steel contains about 97 weight percent iron, 1 weight percent chromium, 0.5 weight percent manganese, 0.3 weight percent carbon and small amounts of other impurities. The Inconel "X" contains about 7 weight percent iron, 75 weight percent nickel and 15 weight percent chromium, plus small amounts of other elements.

The above examples illustrate the results obtained by maintaining the composition of the chemical milling solution constant at certain predetermined values of the concentration of the various components. The phosphorus, chloride ion, nitrate ion and acidic hydrogen concentrations were given in grams per liter. In each case, the balance consisted essentially of water. In the cases in which acceptable results were obtained, the weight ratio of phosphorus-to-metal in solution varied from 0.23 to 1.50; the acidic hydrogen varied from 3.5 to 12.3; the chloride ion concentration varied from 35 grams per liter to 302 grams per liter, and the nitrate ion concentration varied from 80.5 grams per liter to 290 grams per liter.

When the values of either of the weight ratio of phosphorus-to-metal, or, the acidic hydrogen or nitrate ion concentration varied beyond these limits, it was found that poor chemically milled surfaces resulted. For in-

stance, No. 11 in the table illustrates the undesirable effect that an excess of acidic hydrogen has on the chemically milled surface. No. 12 illustrates the bad effect that an excess of nitrate ion has in milling solutions. No. 13, on the other hand, illustrates the disadvantages of using a solution having too little dissolved iron as compared to the amount of phosphorus in solution. Thus, it is seen that a weight ratio of 1.79 of phosphorus-to-metal is too high.

The above examples thus illustrate the advantage that is obtained by using the process of this invention in chemically milling steel and steel alloy workpieces. By keeping the chloride or other halide ion, the nitrate ion and the weight ratio of phosphorus-to-metal in solution within certain predetermined limits, good chemically milled surfaces can be obtained even when the amount of metal removed from the surface of the workpiece is considerable. This uniformity of chemically milled surfaces is of extreme importance in the manufacture of structural metal parts as, for example, in the manufac-

ture of airframe structural panels having maximum strength-to-weight ratios. In the latter instance, the structural panels are preformed to the desired curvature or shape and then the areas undergoing the least mechanical stress are chemically milled out to provide thinner sections.

Besides being able to control the quality of the chemically milled surface, the process has many other advantages. One of these is that the milling solution does not have to be discarded periodically and replaced by a new one as was the case in the prior art processes. This reduction in handling constitutes a considerable saving in both time and the economics of the process. Another advantage of this process is that the disposal problem of waste acids has been overcome since the only by-product is the metal phosphates such as phosphates of nickel iron and chromium, which are removed as a precipitate.

The examples illustrate that certain variations may be made in carrying out the process of this invention, especially in regard to the concentration of the various components of the chemical solution. However, it is seen that certain limits in concentrations of the various ingredients must be maintained since, as seen in No. 13 of the table, for instance, too low a concentration of iron results in an unacceptable chemically milled surface. This example illustrates that one cannot expect to obtain a good chemically milled surface by starting with the solution containing no iron, and carrying out the chemical milling by a batch process since the composition would then be constantly changing so that unpredictable

and unsatisfactory results would be obtained. When, however, the concentrations are maintained constant by a recycling process described in this case, satisfactory and predictable results can be obtained. Certain other variations may be made in carrying out the process of this invention without departing from the spirit and scope of the chemical milling process as described hereinabove. For example, the amount of water that is added to the precipitation container 17 may vary from one to ten times the volume of the phosphates of iron residue admitted from the distillation apparatus 8.

The acids used in this process were commercially available. The phosphoric acid used was either 85 percent acid by weight having a specific gravity of 1.69, or 75 percent acid by weight having a specific gravity of 1.58. The nitric acid employed was 70 percent by weight acid and had a specific gravity of 1.42. Two kinds of hydrochloric acid were used, of which one was 37 percent acid by weight having a specific gravity of 1.18, and the other was 30 percent acid by weight and had a specific gravity of 1.15.

Although the invention has been described and illustrated in detail, it is to be clearly understood that the same is by way of illustration and example only and is not to be taken by way of limitation, the spirit and scope of this invention being limited only by the terms of the appended claims.

I claim:

1. The continuous process of chemically milling workpieces of group VIII metals and alloys thereof comprising exposing a workpiece to the etching action of a bath initially containing dissolved phosphorus and metal in a predetermined weight ratio of from about 0.23 to about 1.50 phosphorus-to-metal, wherein the phosphorus is present in the form of soluble phosphates, withdrawing partially spent portions of said bath containing said dissolved metal and phosphorus, precipitating metal phosphates from said portions to form a precipitate of metal phosphate and an effluent containing metal hydrogen phosphates, returning said effluent to said bath, and adding phosphorus in the form of phosphates to said bath in an amount substantially equivalent to the phosphorus removed in said partially spent portions and maintaining said dissolved metal and phosphorus at said predetermined weight ratio.

2. A continuous process of chemically milling workpieces of group VIII metals and alloys thereof comprising exposing a workpiece to the etching action of a bath initially containing soluble phosphates and metal in a predetermined weight ratio of phosphorus-to-metal, withdrawing partially spent portions of said bath, precipitating metal phosphates from said portions to form a precipitate of metal phosphates and an effluent containing metal hydrogen phosphates, returning said effluent containing metal hydrogen phosphates to said bath, and adding phosphorus in the form of soluble phosphates to said bath in an amount equivalent to the phosphorus removed in said metal phosphate precipitate and maintaining said dissolved metal and phosphorus at said predetermined weight ratio.

3. A process for chemically milling workpieces of group VIII metals and alloys thereof comprising exposing a workpiece to the etching action of a bath initially containing hydrochloric acid, nitric acid, phosphoric acid and dissolved metals wherein the dissolved phosphorus-to-metal weight ratio is from about 0.23 to about 1.50; withdrawing partially spent portions of said bath, precipitating metal phosphates from said portions to form a precipitate of metal phosphates and an effluent containing metal hydrogen phosphates, returning said effluent containing metal hydrogen phosphates to said bath, and adding phosphorus in the form of soluble phosphates to said bath in an amount equivalent to the phosphorus removed in said metal phosphates precipitate and maintain-

ing said dissolved metal and phosphorus at said predetermined weight ratio.

4. The process of claim 3 wherein said bath contains substantially 3.5-12.3 grams per liter of acidic hydrogen, 35.5-302 grams per liter of chloride ion, 80.5-290 grams per liter of nitrate ion, 43-172 grams per liter of phosphorus in the form of soluble phosphates, 30-200 grams per liter of dissolved metal, the balance being substantially water, and wherein the ratio by weight of phosphorus-to-metal in solution is maintained at from about 0.23 to about 1.50.

5. The continuous process of chemically milling workpieces of steel and alloys thereof comprising exposing a workpiece to the etching action of a bath initially containing substantially 3.5-12.3 grams per liter of acidic hydrogen, 35.5-302 grams per liter of chloride ion, 80.5-279 grams per liter of nitrate ion, 43-172 grams per liter of phosphorus in the form of soluble phosphates, 30-200 grams per liter of dissolved metal, the balance being substantially water, and wherein the ratio by weight of phosphorus-to-metal in solution is from about 0.23 to about 1.50, withdrawing partially spent portions of said bath, progressively distilling said withdrawn portions to produce a distillate of water, a distillate of hydrochloric plus nitric acids, and a residue containing phosphates of metal; adding water to said residue to precipitate metal phosphates leaving a liquid phase containing metal hydrogen phosphates, separating said liquid phase from said precipitate, returning said liquid phase containing metal hydrogen phosphates to said bath, and adding phosphorus in the form of soluble phosphates to said bath in an amount equivalent to the phosphorus removed in said metal phosphate precipitate and maintaining said dissolved metal and phosphorus at said predetermined weight ratio.

6. The continuous process of chemically milling workpieces of steel and alloys thereof comprising exposing a workpiece to the etching action of a bath initially containing substantially 3.5-12.3 grams per liter of acidic hydrogen, 35.5-302 grams per liter of chloride ion, 80.5-279 grams per liter of nitrate ion, 43-172 grams per liter of phosphorus in the form of soluble phosphates, 30-200 grams per liter of dissolved metal, the balance being substantially water, and wherein the ratio by weight of phosphorus-to-metal in solution is from about 0.23 to about 1.50, withdrawing partially spent portions of said bath, progressively distilling said withdrawn portion to produce a distillate of water, a distillate of hydrochloric plus nitric acids, and a residue containing phosphates of metal; adding water to said residue to precipitate metal phosphates leaving a liquid phase containing metal hydrogen phosphates, separating said liquid phase from said precipitate, concentrating said liquid phase containing said metal hydrogen phosphates by removing excess water, returning said liquid phase containing metal hydrogen phosphates to said bath, and adding phosphorus in the form of soluble phosphates to said bath in an amount equivalent to the phosphorus removed in said metal phosphates precipitate and maintaining said dissolved metal and phosphorus at said predetermined weight ratio.

7. The process of claim 6 and in addition the steps of adding chloride ion, nitrate ion and water to said bath in an amount substantially equivalent to that lost in carrying out said process.

8. The process of chemically milling a metallic material selected from the class consisting of a group VIII metal and an alloy of a group VIII metal and by subjecting said metallic material to the action of a bath initially containing hydrochloric, nitric and phosphoric acids and dissolved metal wherein the phosphorus-to-metal weight ratio is maintained within a predetermined range of values; the steps of withdrawing partially spent portions of said bath containing dissolved phosphates and metal, distilling off the unused acids leaving metal phosphates and metal hydrogen phosphates in solution,

diluting said solution and thereby precipitating metal phosphates and leaving metal hydrogen phosphates in solution, returning the metal hydrogen phosphates to the bath to maintain said phosphorus-to-metal weight ratio.

9. The process of chemically milling group VIII metals and alloys thereof by subjecting said metals and alloys to the action of a bath initially containing hydrochloric, nitric and phosphoric acids, and dissolved metal in amounts sufficient to maintain a phosphorus-to-metal weight ratio of from about 0.23 to about 1.50, the steps of withdrawing partially spent portions of said bath containing dissolved phosphates and metal, distilling off the unused hydrochloric and nitric acids leaving metal phosphates and metal hydrogen phosphates, diluting said phosphates and thereby precipitating metal phosphates leaving metal hydrogen phosphates in solution, and returning the metal hydrogen phosphates to said bath to maintain said phosphorus-to-metal weight ratio.

10. The process of chemically milling group VIII metals and alloys thereof by subjecting said metals to the action of a bath initially containing from about 35.5-302 grams per liter of chloride ion, 80.5-290 grams per liter of nitrate ion, 43-172 grams per liter of phosphorus in the form of soluble phosphates, 30-200 grams per liter of dissolved metal, the balance being substantially water and wherein the ratio by weight of phosphorus-to-metal is from about 0.23 to about 1.50, the steps of withdrawing partially spent portions of said bath, distilling off the unused hydrochloric and nitric acids leaving metal phosphates and metal hydrogen phosphates, diluting said phosphates and thereby precipitating metal phosphates leaving metal hydrogen phosphates in solution, and returning the metal hydrogen phosphates to the bath to maintain said phosphorus-to-metal weight ratio, and adding phosphorus in the form of phosphates to said bath in an amount substantially equivalent to the phosphorus removed in the form of metal phosphates.

11. The process of claim 10 and in addition the steps of adding chloride ion, nitrate ion and water to said bath in an amount substantially equivalent to that lost in carrying out said process.

12. The process of chemically milling a metallic material selected from the class consisting of a group VIII metal and an alloy of a group VIII metal by subjecting said metallic material to the action of a bath initially containing substantially 92 grams per liter of chloride ion, substantially 148 grams per liter of nitrate ion, substantially 113 grams per liter of phosphorus in the form of soluble phosphates, substantially 106 grams per liter of dissolved metal, the balance being substantially water and wherein the ratio by weight of phosphorus-to-metal is substantially 1.08, the steps of withdrawing partially spent portions of said bath, distilling off the unused hydrochloric and nitric acids leaving a residue of metal phosphates and metal hydrogen phosphates, adding water to said phosphates and thereby precipitating metal phosphates leaving metal hydrogen phosphates in solution, returning said metal hydrogen phosphates to said bath and adding phosphorus in the form of soluble phosphates to said bath in an amount substantially equivalent to the phosphorus removed in the form of metal phosphates to maintain said phosphorus-to-metal weight ratio and adding chloride ion, nitrate ion and water in an amount substantially equivalent to that lost in carrying out said process.

13. The process of chemically milling a metallic material selected from the class consisting of nickel and an alloy of nickel by subjecting said metallic material to the action of a bath initially containing substantially 153 grams per liter of chloride ion, substantially 290 grams per liter of nitrate ion, substantially 68 grams per liter of phosphorus in the form of soluble phosphates, substantially 76 grams per liter of dissolved metal, the balance being substantially water and wherein the ratio by weight of phosphorus-to-metal is substantially 0.90,

the steps of withdrawing partially spent portions of said bath, distilling off the unused hydrochloric and nitric acids leaving a residue of metal phosphates and metal hydrogen phosphates, adding water to said phosphates and thereby precipitating metal phosphates leaving metal hydrogen phosphates in solution, returning the metal hydrogen phosphates to said bath and adding phosphorus in the form of phosphates to said bath in an amount substantially equivalent to the phosphorus removed in the form of metal phosphates to maintain said phosphorus-to-metal weight ratio.

14. A continuous process for chemically milling a workpiece selected from the class consisting of steel and an alloy of steel comprising exposing said workpiece to the etching action of a bath initially containing substantially 9.6 grams per liter of acidic hydrogen, substantially 92 grams per liter of chloride ion, substantially 148 grams per liter of nitrate ion, substantially 113 grams per liter of phosphorus in the form of soluble phosphates, substantially 106 grams per liter of dissolved metal, the balance being substantially water, and wherein the ratio by weight of phosphorus-to-metal in solution is substantially 1.08, withdrawing partially spent portions of said bath; progressively distilling said withdrawn portions to produce a distillate of water, a distillate of hydrochloric and nitric acids, and a residue containing phosphates of metal; adding water to said residue and thereby precipitating metal phosphates leaving a liquid phase containing metal hydrogen phosphates, separating said liquid phase from said precipitate, concentrating said liquid phase containing said metal hydrogen phosphates by removing excess water, returning said concentrated liquid phase containing metal hydrogen phosphates to said bath, adding phosphorus in the form of soluble phosphates to said bath in an amount equivalent to the phosphorus removed in said metal phosphate precipitate and maintaining said phosphorus-to-metal in said bath at said predetermined weight ratio; and adding chloride ion, nitrate ion and water to the said bath in an amount substantially equivalent to that lost in carrying out said process.

15. A continuous process for chemically milling a workpiece selected from the class consisting of nickel and an alloy of nickel comprising exposing said workpiece to the etching action of a bath initially containing substantially 3.5-12.3 grams per liter of acidic hydrogen, 35.5-302 grams per liter of chloride ion, 80.5-290 grams per liter of phosphorus in the form of soluble phosphates, 30-200 grams per liter of dissolved metal, the balance being substantially water, and wherein the ratio by weight of phosphorus-to-metal in solution is within the range of values of from about 0.23 to about 1.50, withdrawing partially spent portions of said bath; progressively distilling said withdrawn portions to produce a distillate of water, a distillate of hydrochloric plus nitric acids, and a residue containing phosphates of metal; adding water to said residue and thereby precipitating metal phosphates leaving a liquid phase containing metal hydrogen phosphates, separating said liquid phase from said precipitate, returning said liquid phase containing metal hydrogen phosphates to said bath, and adding phosphorus in the form of soluble phosphates to said bath in an amount equivalent to the phosphorus removed in said metal phosphate precipitate, and maintaining said phosphorus-to-metal ratio in solution within said range of values.

16. A continuous process for chemically milling a workpiece selected from the class consisting of nickel and an alloy of nickel comprising exposing said workpiece to the etching action of a bath initially containing substantially 11.5 grams per liter of acidic hydrogen, substantially 153 grams per liter of chloride ion, substantially 290 grams per liter of nitrate ion, substantially 68 grams per liter of phosphorus in the form of soluble phosphates, substantially 76 grams per liter of dissolved metal, the balance being substantially water, and wherein the ratio

by weight of phosphorus-to-metal in solution is substantially 0.9, withdrawing partially spent portions of said bath; progressively distilling said withdrawn portions to produce a distillate of water, a distillate of hydrochloric plus nitric acids, and a residue containing phosphates of metal; adding water to said residue and thereby precipitating metal phosphates leaving a liquid phase containing metal hydrogen phosphates, separating said liquid phase from said precipitate, concentrating said liquid phase containing said metal hydrogen phosphates by removing excess water, returning said concentrated liquid phase containing said metal hydrogen phosphates to said bath, and adding phosphorus in the form of soluble phosphates to said bath in an amount equivalent to the phosphorus re-

10

moved in said phosphate metal precipitate, and maintaining said ratio by weight of phosphorus-to-metal in said bath.

17. The process of claim 16 and in addition the steps of adding chloride ion, nitrate ion and water to said bath in an amount substantially equivalent to that lost in carrying out said process.

## References Cited in the file of this patent

## UNITED STATES PATENTS

|           |          |               |
|-----------|----------|---------------|
| 2,235,658 | Waterman | Mar. 18, 1941 |
| 2,337,062 | Page     | Dec. 21, 1943 |
| 2,662,814 | Swihart  | Dec. 15, 1953 |